

# UNITED STATES PATENT OFFICE.

FREDERIC E. CARTER, OF NEWARK, NEW JERSEY, ASSIGNOR TO BAKER & COMPANY, INC., A CORPORATION OF NEW JERSEY.

## ALLOY.

1,378,996.

Specification of Letters Patent. Patented May 24, 1921.

No Drawing.

Application filed July 17, 1920. Serial No. 396,930.

To all whom it may concern:

Be it known that I, FREDERIC EDWARD CARTER, a subject of Great Britain, and a resident of Newark, in the county of Essex and 5 State of New Jersey, have invented new and useful Improvements in Alloys, of which the following is a specification.

This invention relates more particularly to an alloy to replace platinum-iridium, as it 10 is employed for hypodermic needles, magneto contacts and the like, and the objects of the invention are to avoid the use of iridium, which is expensive and difficult to obtain; to obtain an alloy which shall closely 15 simulate platinum-iridium in all the qualities which render it especially adapted to the uses for which it is employed; to obtain a practicable facility in working the alloy, and to obtain other advantages and results 20 as may be brought out in the following description.

In carrying out my invention I form an alloy of gold and palladium with an excess of platinum, by fusing or melting them together 25 and the proportions of such metals which I use are substantially  $\frac{1}{2}\%-5\%$  of palladium and 5%-15% of gold, the rest of

the alloy being platinum. While it has been long known that small quantities of gold added to platinum increase its hardness, it 30 has also been well-known that not more than about 9% of gold could be added without the resulting alloy becoming too brittle to be workable. I have discovered that the addition of a small quantity of palladium will 35 avoid this difficulty and produce a workable alloy even if considerable more gold than 9% is employed. The gold secures hardness in my new alloy, while the palladium avoids brittleness and makes the alloy 40 workable, and it will be understood from this that the proportions of the metals can be varied to adapt the alloy to different purposes or uses, without departing from the spirit and scope of the invention, and I 45 do not wish to be understood as restricting myself except as the state of the art may require.

Having thus described my invention, what I claim is:

An alloy containing substantially  $\frac{1}{2}\%-5\%$  palladium, 5%-15% gold and the rest platinum.

FREDERIC E. CARTER.